

May 26, 1936.

A. B. KINZEL

2,042,427

## APPARATUS FOR USE AT LOW TEMPERATURES

Original Filed March 11, 1933



## INVENTOR

INVENTOR  
Augustus B. Kenzel  
BY  
Watson, Bristol, Johnson & Leavenworth  
ATTORNEYS

## UNITED STATES PATENT OFFICE

2,042,427

## APPARATUS FOR USE AT LOW TEMPERATURES

Augustus B. Kinsel, Flushing, N. Y., assignor, by  
mesne assignments, to Union Carbide and  
Carbon Corporation, a corporation of New  
York

Original application March 11, 1933, Serial No.  
660,365. Divided and this application Febru-  
ary 5, 1934, Serial No. 709,718

1 Claim. (CL 220—8)

This invention relates to apparatus for use at low temperatures, and particularly to apparatus including containers or vessels for holding liquefied gases, for example liquid air or oxygen, and to the construction of the same whereby a metal or alloy is employed that is not embrittled at the low temperatures encountered.

The invention has for its object generally the provision of improved apparatus of the character indicated which is strong and durable both at atmospheric temperatures and at the temperatures of the liquefied gas being handled, for example at the temperature of liquid air or oxygen.

It is also an object to provide improved apparatus such as containers for handling liquefied gases fabricated of an alloy that is characterized by the possession of mechanical strength and ductility and relatively high Izod values when subjected to impact at very low temperatures.

Still another object is to provide improved compositions for alloys for use in apparatus of the character indicated which do not have notch-brittleness at very low temperatures, for example at  $-150^{\circ}$  C. or  $123^{\circ}$  Kelvin (hereinafter denoted degrees K.), and which are free from internal stresses at such low temperatures.

Other objects of the invention will in part be obvious and will in part appear hereinafter.

The invention accordingly comprises the features of construction, combination of elements, and arrangement of parts, which will be exemplified in the construction hereinafter set forth and the scope of the application of which will be indicated in the claims.

This application is a division of my application Serial No. 660,365, filed March 11, 1933.

For a fuller understanding of the nature and objects of the invention, reference should be had to the following detailed description taken in connection with the accompanying drawing, in which:

The figure depicts exemplary apparatus in vertical cross-section, particularly a container for liquid oxygen, made in accordance with the invention.

It is generally impracticable to confine large quantities of liquefied gases of the character indicated in completely closed vessels, though it is possible to confine them within pressure vessels or containers provided with relief valves or other means for preventing the building up of excessive pressures. When this is done, gas pressures of the order of 100 pounds per square inch and above may be safely attained within the apparatus. Considerable difficulty, however, is involved in

finding a material suitable for use in the construction of such apparatus.

Heretofore, two materials have generally been employed, such as steel and copper. The disadvantage in the use of steel is that it becomes exceedingly brittle at temperatures below about  $223^{\circ}$  K. (or  $-50^{\circ}$  C.). If there are any locked-up stresses in the articles, due to the conditions of fabrication, the additional stresses set up during the chilling of the article to the temperature of liquid oxygen may be sufficient to cause the failure of the embrittled steel. For this reason, very careful annealing has been practiced in making such apparatus. Even if such annealing is employed and all locked-up stresses are removed, however, the extreme brittleness of the steel renders it highly sensitive to shock and vibration at these low temperatures. For this reason, the steel article must be specially supported to minimize the danger of shock vibration.

Copper has the advantage of remaining ductile at the temperatures encountered in dealing with liquefied gases of the character indicated. Copper, however, has serious disadvantages, in that, if free from strains, it has practically no plastic-free elasticity and does not completely return to shape after the removal of an imposed stress. It gradually stretches with a corresponding reduction in cross-section. Thus, if a vessel of copper or other article of such composition becomes deformed, a failure may occur when it is again put under pressure which it could safely have withstood when new. To avoid this sort of failure, it has been proposed to measure the article under stress, but this is not always practical, and in any event a deformed vessel is no longer suitable for its original purpose.

In the practice of the present invention, preferably those parts of the apparatus which are subject both to stress and a very low temperature are made of a metal alloy having substantial freedom from internal stress at such temperature. Referring to the drawing, 10 denotes a thick-walled outer vessel of containing apparatus for liquefied gases, which may be made of welded metal sections, and has a spaced inner lining or basket 11 which holds a body 12 of the liquefied gas, for example, liquid oxygen. The vessel is provided with suitable fluid manipulating connections, for example, a gas-phase withdrawal connection 13 and a liquid-phase withdrawal connection 14, together with a filling connection, as shown at 15.

The vessel 10 is preferably enveloped with heat insulating material, as shown at 16, and has a

supporting casing 17, supporting connections with the casing being provided in any suitable manner, for example by means of cables or chains 18, of relatively poor heat conductivity, which are anchored at one end to the casing and at the other to a ring 19 that embraces the vessel. In the apparatus illustrated, the vessel 16, and such other parts as may be desired are fabricated of a metal alloy having substantial freedom from internal stress at the temperature of liquid oxygen.

A metal alloy, which has the desired freedom from internal stresses and is suitable for making such vessel and other desired parts, may be prepared in a variety of ways, for example, by dispersing a small amount of a component in a main metallic mass possessing the desired ductility, the dispersion being such as to interfere with the normal slip of the planes of the main metallic lattice when subject to stress. This effects strengthening of the lattice. When the precipitated particles are sufficiently fine, local stresses produced by temperature changes from room temperature to a temperature of liquid oxygen are not sufficient to produce brittleness. If, however, a combination of extremely fine and moderately fine particles is considered, the local stresses are sufficient to affect seriously the low temperature ductility.

30. A second way of accomplishing the desired strengthening of non-ferrous materials without necessarily high internal stress, local or otherwise, is to introduce a foreign element into the metallic matrix so that it is in solid solution; that is, it either replaces one of the atoms of the matrix material in the lattice or associates itself by means of electronic bonds to form a group of one or more metallic atoms which may form a secondary lattice, superimposed on the primary lattice. Again interference with normal slip is affected and the material is strengthened. In this type, it is most probable that temperature stresses will not be present because of the homogeneous distribution of the two or more types of atoms involved.

50. It has generally been found in non-ferrous metallurgical practice that when a given strengthening mechanism is relied on for more than a relatively small increase, secondary effects take place. The embrittlement of duralumin or nickel-silicide-copper, when the precipitation effect is employed for maximum strength, is a case in point, as the ductility is very adversely affected, and it is necessary to limit the strength to an optimum amount to get the desired ductility. Solid solution phenomena are also limited in scope, as frequently if an increase in the amount of foreign atoms is introduced, the tendency to compound formation increases with consequent rapid falling off of ductility with increased strength. The oldest recognized method of strengthening metals consists in forming eutectics by means of a second component. Eutectics, in general, will not fill the needs of the alloy in the invention because the heterogeneous nature of a lamellar structure tends to promote local thermal stresses at low temperatures. However, a comparatively small amount of suitable eutectic may be formed without deleterious effect if the solid solution matrix is the predominately continuous phase.

70. According to the present invention, an alloy is produced in which the strength is higher than that obtained by any one of the above described ways, particularly with respect to ductility and

with respect to elimination of thermal stress when the alloy is cooled to liquid oxygen temperature; the alloy here provided comprising elements so combined that two or more of the aforementioned desired effects are simultaneously obtained.

The main metallic component of the composition used in the present invention thus is a metal which has high ductility throughout substantially the whole range of service temperatures, for example from 100° C. down to and including that of the liquefied low boiling point gases. This is particularly true of the non-ferrous empirical group of metals comprising copper, aluminum, and magnesium. Such metallic component is taken in an amount comprising generally more than 90% by weight of the whole metallic composition. Certain alloys of the group are also suitable for the main component or matrix metal, as are combinations within the above group constituting 90% of the matrix. Zinc brasses or aluminum bronzes, which are chiefly copper, are illustrative. As a specific example may be mentioned a brass which has as its components copper and zinc taken in substantially the ratio of six parts of copper to four parts of zinc.

As a second component for the metallic composition adapted to form a solid solution with the main metallic component there is employed a metalloid or metallic element, which forms a solid solution with the first in the manner of the well known binary systems. A suitable component of this character for the compositions desired may be chosen from the empirical group consisting of boron, silicon, and beryllium. Silicon is preferable because it tends to form compounds with a third metallic component, hereinafter described, when taken in relatively small amounts, for example 3% of silicon begins to 40 form a eutectic with magnesium, 5% with copper and 1.6% with aluminum. Beryllium forms a solid solution with copper up to 2.8%, but more than these amounts form the eutectic.

A third component may be employed for a composition of metal made according to the present invention, such component being of a character such that it remains in dispersion throughout the metallic mass, either in atomic form or as a compound with the main combination or one of the secondary combinations and by means of this dispersion effects interference with the slip of the metallic planes in the metallic lattice as previously described. A suitable component for accomplishing this is chosen from the empirical group consisting of manganese, iron, nickel, and chromium. Manganese is generally preferable because of its action in the metallic bath when preparing the alloy. The manganese is taken in relatively small amounts; for example 60 in amounts approximating not over 4% by weight of the total mass, which is also true for iron and nickel. Chromium, however, should be taken generally in smaller amounts; for example, in amounts in the neighborhood of 2% by weight 65 of the total mass.

The functions of the metals chosen for first and second additions may overlap, that is, the main solid solution alloying element may tend to give precipitation when taken in certain amounts and under certain conditions of heat treatment. Beryllium is an illustration when used with copper. Amounts in excess of the solid solution saturation content at room temperature may be used in dispersion strengthening. Likewise,

wise, the elements of the second group all form solid solutions with copper to more or less limited extent.

Moreover, it is possible and may be desirable 5 to employ elements selected from any of these groups to promote strengthening to a limited degree by taking them in such amounts as to cause the presence of eutectics, the relative proportion being substantially small when compared to the 10 amount of base metal matrix used. Generally, however, this is not desirable, as eutectics are conducive to the production of thermal stresses at low temperatures.

The following are examples of compositions 15 made in accordance with the invention:

*Example I*

|           | Percent |
|-----------|---------|
| Copper    | 96      |
| Silicon   | 3       |
| Manganese | 1       |

*Example II*

|           | Percent |
|-----------|---------|
| Copper    | 58      |
| Zinc      | 38      |
| Silicon   | 3       |
| Manganese | 1       |

*Example III*

|           | Percent |
|-----------|---------|
| Magnesium | 98.4    |
| Silicon   | 1.2     |
| Manganese | .4      |

*Example IV*

|         | Percent |
|---------|---------|
| Copper  | 97.1    |
| Silicon | .4      |
| Nickel  | 2.5     |

*Example V*

|          | Percent |
|----------|---------|
| Copper   | 98.7    |
| Silicon  | .3      |
| Chromium | 1.0     |

*Example VI*

|           | Percent |
|-----------|---------|
| Aluminum  | 92.5    |
| Beryllium | 1.5     |
| Iron      | 3.0     |
| Manganese | 3.0     |

*Example VII*

|           | Percent |
|-----------|---------|
| Copper    | 94      |
| Beryllium | 6       |

When tests are made to compare the physical properties of alloys of the above compositions with those of steel, standard specimens are prepared and placed in a testing machine where the ultimate strength is determined both at room temperature and at the temperature to which it will be subjected when in use, for example at 90° K. The yield point is similarly ascertained, together with the elongation and the reduction in area. When a standard specimen of an alloy of the composition of Example I is made comparatively with one of steel having the composition: carbon 0.40%; manganese 0.68%; silicon 0.28%; phosphorous 0.01%; sulphur 0.30%; the remainder being iron; typical values of these

tests are obtained which are comparatively set forth in the following table:

| Physical property             | Steel      |           | Typical alloy |           |
|-------------------------------|------------|-----------|---------------|-----------|
|                               | Room temp. | At 90° K. | Room temp.    | At 90° K. |
| Ultimate strength lb./sq. in. | 94,360     | 142,800   | 58,200        | 83,300    |
| Yield point lb./sq. in.       | 60,210     | 136,000   | 25,000        | 33,500    |
| Percent elongation            | 28.5       | 7.5       | 69.0          | 84.0      |
| Percent reduction in area     | 52.0       | 8.2       | 77.0          | 70.0      |

Tests on an alloy of the composition of Example I when subject to Izod impact tests show values at room temperatures of from 58 to 64 foot-pounds, while at the low temperature of 90° K. values of from 70 to 78 foot-pounds are obtained. Similar tests with steel of the above composition show Izod values of from 35 to 45 foot-pounds at room temperature, while at 90° K. it gave substantially zero values and shattered easily.

Besides high Izod test values, an alloy of the composition of Example I has additionally the desirable properties of great ductility and workability, weldability with great strength and toughness of welds, and relatively low heat conductivity as compared with copper; this latter being in general a property in common with all the alloys proposed in accordance with the invention.

Izod values of the order of 40 foot-pounds are had from standard specimens of an alloy of the composition of Example II at temperatures in the neighborhood of that of liquid air, the alloys of the other examples giving similar substantial values at temperatures in the neighborhood of that of liquid air.

From the above, it will be seen that the criterion of strength is the usual tensile test and that the criterion for ductility which postulates the absence of internal stresses at low temperature is the Izod value obtained at such temperatures. Hence, it is seen from the above that the alloys here proposed for use in apparatus which is subjected to stress and very low temperatures provide safe apparatus that is substantially free from internal stresses in the metal composing it when subject to a low temperature such as that of liquid air or oxygen.

Since certain changes may be made in the above construction and different embodiments of the invention could be made without departing from the scope thereof, it is intended that all matter contained in the above description or shown in the accompanying drawing shall be interpreted as illustrative and not in a limiting sense.

Having described my invention, what I claim as new and desire to secure by Letters Patent, is:

Apparatus for use in storing, transporting and dispensing liquid oxygen comprising a relatively thick-walled pressure vessel having a heat insulating envelope and support therefor, and subject to a temperature in the neighborhood of 90° K., said vessel being made of sections joined together in a fabricated whole and of an alloy which consists of copper taken in an amount in excess of 90% by weight of the whole, the balance being beryllium; the copper and beryllium being so combined and compounded as to impart to the alloy relatively great mechanical strength, substantial absence of internal stress, and a relatively high Izod value when at said low temperature in comparison with such properties at room temperature.

AUGUSTUS B. KINZEL 75